

J. C. ADELL.

METHOD OF SEPARATING THE OXIDS OF IRON AND OTHER METALS OCCURRING IN COMPOUND ORES.  
APPLICATION FILED DEC. 2, 1916.

1,318,431.

Patented Oct. 14, 1919.



Inventor

James Claude Adell  
By Hull, Smith, Brock, & West  
Atty's.

# UNITED STATES PATENT OFFICE.

JAMES CLAUDE ADELL, OF CLEVELAND, OHIO.

## METHOD OF SEPARATING THE OXIDS OF IRON AND OTHER METALS OCCURRING IN COMPOUND ORES.

1,318,431.

Specification of Letters Patent. Patented Oct. 14, 1919.

Application filed December 2, 1916. Serial No. 134,583.

To all whom it may concern:

Be it known that I, JAMES CLAUDE ADELL, a citizen of the United States, residing at Cleveland, in the county of Cuyahoga and State of Ohio, have invented a certain new and useful Improvement in Methods of Separating the Oxids of Iron and other Metals Occurring in Compound Ores, of which the following is a full, clear, and exact description, reference being had to the accompanying drawings.

This invention relates to a method of separating iron containing compounds from other minerals such as manganese dioxid, occurring in compound ores, and the object of the invention is the provision of a process whereby this separation can be effected in a simple, rapid, and inexpensive manner.

Iron ores bearing manganese dioxid up to 20 as much as 20 per cent. of the latter are ordinarily worth only from \$1.00 to \$1.25 per ton more than iron ore having no manganese. At the same time the manganese dioxid or reasonably pure pyrolusite is worth 25 on the market from \$200.00 to \$300.00 per ton, this remarkable condition being due to the expense incident to practising previously known methods of separating the ingredients.

According to my improved method I first pulverize the ore thoroughly and subject it to the action of steam or water vapor while keeping it at an elevated temperature, say 600° to 800° C. Most iron ore consists 35 largely of hematite having a formula of approximately  $Fe_2O_3 \cdot 6H_2O$ . Roasting this ore in the presence of steam changes it to  $Fe_3O_4$ , which as is well known, is magnetic. Besides this material emerges from the process 40 in a dry, light, finely divided condition which is peculiarly adapted for the magnetic separation process. The manganese dioxid emerges from the process unchanged, although whether or not it has any action 45 on the process I cannot say, although it is a peculiarly active catalytic agent in many relations. Also I do not assert any theory as to the reactions taking place but relate merely the observed results of the manipulations described.

The separation of the magnetic oxid from the non-magnetic materials may be effected by the gravity process, by dropping the treated material past the face of magnets, 50 which deflect the iron containing materials

slightly out of the perpendicular path leaving the non-ferruginous parts unaffected. Any gangue present in the ore will remain unaffected either by the roasting operation or by the magnetic separation, and must be 60 removed from the pyrolusite or other mineral subsequent to this separation. The magnetic oxid, when compressed into briquets, becomes a very valuable source of iron, since owing to its purity, iron of great 65 purity can be produced therefrom.

The particular ore upon which I have performed this process is one consisting approximately of  $Fe_2O_3$ , 80 to 88 per cent.;  $MnO_2$ , 20 to 12 per cent. The specific gravities of the two minerals differ only by a few tenths of one per cent., which is too small to 70 permit of separation by ordinary processes.

In the drawing accompanying and forming a part of this application, wherein I 75 have illustrated one form of apparatus whereby my invention may be carried out, Figure 1 represents a longitudinal sectional view through the kiln and showing the magnetic separator in elevation, and Fig. 2 a 80 cross sectional view on the line 2—2 of Fig. 1.

Describing the parts by reference characters, 1 represents an elongated rotatable cylindrical kiln having the usual tires 2, 2 85 running upon the supporting wheels 3, 3, one of which is driven by gearing 4. Surrounding the mid-portion of the kiln is a housing 5 having at one end a furnace 6 and at the other end a flue or stack 7. The ends 90 of the kiln project into shields or chambers 8, 9 respectively, both of which make fairly close joints with the kiln exterior. Carried by the shield 8 is the inlet hopper 10 to which the pulverized ore is delivered, and 95 from which it is fed in a gradual uniform manner by suitable means such as the worm 11 driven by the shaft 12. The material delivered from the kiln into the shield 9 is also removed therefrom by suitable means such 100 as the worm 13 driven by the shaft 14. The shafts 12 and 14 are preferably operatively connected as by a shaft 15 geared thereto so that the worms will be operated at the same speed. In addition to their convenience and 105 simplicity, worms such as here shown have the advantage that they tend to prevent the inlet or escape of gases while providing for the free measured escape of solids.

A steam pipe 16 controlled by a valve 17 110

projects into the lower end of the kiln and may be terminated in a suitable spray head 18. In fact all of the air necessary for the combustion can very conveniently be delivered in this way, the indraft produced at the various crevices and joints through the agency of the stack 7 serving to prevent the loss of steam therefrom; while the warm mixture of steam and air drawn through 10 the pipe 19 produces efficient combustion.

The material delivered by the worm 13 flows through the conduit 20 to a suitable spreading table 21 from which it falls in a fine sheet past the end of a suitable magnet 15 22 which permits the non-ferruginous materials to fall freely into the bin 23, while the magnetic particles are deflected into the bin 24.

For the treatment of hematite ores, the 20 roasting is effected in a non-oxidizing atmosphere, but for sulfur containing ores it is necessary first to roast in air so as to drive off the sulfur and oxidize the ore, after which the same process is performed as in 25 the case of hematite.

I am aware that the heat can be provided, either by internal or external combustion and that in a large plant it may be desirable to pass the furnace gases through the kiln 30 instead of around the same; although for smaller operations I have employed the arrangement shown with excellent results and prefer this mode, partly by reason of the greater purity of the product and the smaller

waste of steam and the greater rapidity of 35 the reaction which is blanketed to some extent by the reducing gases of the furnace when they are admitted inside the kiln.

While I have specifically described my invention in connection with the separation 40 of hematite from pyrolusite, it will be understood that I do not confine myself to this particular use but propose the same equally for ores of iron containing other minerals.

Having thus described my invention, 45 what I claim is:—

1. The method of recovering pyrolusite from a mixed ore of hematite and pyrolusite which consists in first pulverizing the ore, second roasting the same in the presence 50 of water vapor whereby the hematite is changed to magnetic oxid, and third removing said magnetic oxid magnetically from the unchanged pyrolusite.

2. The process of recovering pyrolusite 55 from a mixture of pyrolusite and hematite which consists in roasting the pulverized mixed substances to a low red heat in a current of water vapor and thereafter separating the resulting magnetic oxid magneti- 60 cally from the unchanged pyrolusite.

In testimony whereof, I hereunto affix my signature in the presence of two witnesses.

JAMES CLAUDE ADELL.

Witnesses:

KATE R. ADELL,  
ETHEL B. ADELL.